

Nov. 19, 1940.

W. C. ROBINSON ET AL

2,222,556

ELECTRICAL CONDUCTOR

Filed Aug. 18, 1939



INVENTORS  
William C. Robinson, and  
Ralph W. E. Moore  
by Christy and Walton  
attorneys.

## UNITED STATES PATENT OFFICE

2,222,556

## ELECTRICAL CONDUCTOR

William C. Robinson, Sewickley, Pa., and Ralph W. E. Moore, Riverdale, N. Y., assignors to National Electric Products Corporation, a corporation of Delaware

Application August 18, 1939, Serial No. 290,862

3 Claims. (Cl. 174—122)

This invention relates to an insulated conductor.

We have discovered that in the manufacture of insulated conductors great advantage is derived both in the manufacture and also in the qualities and useful life of an insulated conductor by replacing the braided or woven fibrous covering which previously has been commonly applied around the core of the conductor by a serving of fibrous material, such as cotton strand, wound on the conductor core in a simple helical lay with its turns in intimate contact with each other, and bound together against opening tendencies during the flexion of a conductor by a binder filament or filaments. Further we have discovered that if the binder filament or filaments, which are laid in a helix opposite in sense to the helical lay of the absorbent strands, are laid to form a sufficiently great angle with respect to the longitudinal axis of the conductor, or with respect to the angle at which the served covering is laid, the binder filament, though of commonly used material and much lighter in gauge than the serving strands, tends remarkably well to resist breakage under severe flexion of the conductor. These discoveries we have disclosed and claimed in our co-pending applications Serial No. 181,910, filed December 27, 1937, and Serial No. 224,522, filed August 12, 1938; of which applications this forms a continuation-in-part.

We have further discovered that great advantage is to be derived in the insulated conductor assembly by using a binder filament having an extensibility greatly exceeding the extensibility of cotton, and which because of such extensibility, coupled with superior strength, simplifies the manufacture and improves the qualities of the insulated conductor as a whole.

It should be explained that in an insulated conductor in which the fibrous covering of the conductor core is served, there is a strong tendency for the turns of the serving to open up by separation from each other under severe flexion, or kinking, of the conductor. When the turns so open up, the continuity of the moisture-resistant and flame-retardant material with which they are saturated is broken, and the encapsulation provided by the overlying coating of such material and any further coatings, such as coating of paint and wax, is also broken. The protective effect of the fibrous covering of the conductor core is thus destroyed, since air and moisture may penetrate into the interior of the conductor structure in the region of the disintegra-

tion, and the flame-retardant elements of the structure are interrupted. This in the past has proven obstructive to the practice of serving absorbent material around the inner elements, or core, of insulated conductors, although a simple serving tends to form a better seal when impregnated with a viscous saturant, and thus provides a covering less pervious to the entry of air or moisture and of better insulating qualities than does a braided covering. Also it does not tend, as does a braid, to entrap air, the presence of which in contact with a rubber sheath in a conductor tends ultimately to cause deterioration of the rubber.

It is the opening tendency between the turns of a served covering or wrap which a binder filament prevents, and the integration of the insulating structure is thus no greater than the effectiveness of the binder. It may be noted that even in insulated conductors which comprise two coverings or wraps served oppositely to each other, an opening between the turns of the outer wrap when the conductor is severely flexed, or kinked, serves to disintegrate the insulating structure of the conductor, and a suitably organized binder filament is nonetheless essential to counteract such opening tendency.

With the above explanation, it will be readily understood that in an insulated conductor in which dependence is placed upon a served and bound fibrous covering, rather than upon a fibrous covering which is braided or woven, the assembly as a whole effectively possesses an endurance as an adequately insulated conductive assembly directly dependent upon the ability of the binder filament enduringly to lock in close contact with each other the turns of the served wrap, or the outermost served wrap, of the conductor assembly.

In the accompanying drawing Fig. I is a plan view or elevation of the interior assembly of an insulated conductor made in accordance with the structural arrangement of which our invention is incorporated; this figure of the drawings showing a conductor of relatively small size, such as a conductor smaller than a No. 6 size. Fig. II is a generally similar view which, however, shows the internal assembly of a conductor, of a No. 6 size, or greater. Fig. III is a view of a completed insulated conductor including the internal assembly shown in Fig. I, the conductor being shown partly in elevation or plan view or partly in central longitudinal section. Fig. IV is a fragmentary central longitudinal sectional view of the conductor assembly shown in Fig. I, 55

illustrating the structure on an enlarged scale. Fig. V is a cross-sectional view through the conductor shown in Fig. IV.

In Fig. I of the drawing, reference numeral 1 designates the metallic conductive element of the conductor assembly. This conductive element 1 is shown as a single wire of copper, or the like, but may, if desired, be a conductive element of the stranded sort known to the trade as a "flexible" conductor. The metallic conductive element 1 is, as shown, surrounded directly by a one-piece sheath 2 of rubber, or rubber composition, and this innermost assembly of metallic conductive element or sheath is usually termed 10 the core of the conductor consistently with our invention, this core may consist of the metallic conductive element covered with an impregnated braid or other material, or may consist merely of the metallic conductive element itself. There 15 is helically wound or served a wrap of absorbent fibrous material, such as cotton strands. This wrap or serving 3 is shown in Figs. I and II as being served with the simultaneous application of eight "ends" or individual strands, the more 20 rapidly to effect the serving. Also, the more rapidly to effect the serving and the more coherently to apply the wrap, the strands are served with a substantial lead, being shown as applied at an angle  $a$  of about 50 degrees to the 25 longitudinal axis of the conductor.

The binder filament 4 is applied wholly outside the serving 3 and is laid in a helix opposite to that in which the serving is laid, so that the turns of the open binder structure cross, and bind 30 together, the turns of the serving. As above explained, the function of this open binder structure is to bind the turns of the serving against a separation from each other which would destroy the integration of the insulating and protective 35 assembly outwardly of the core, and in order to perform this function, it is necessary that the binder filament (by which term we intend to include any number of filaments which form an open structure) should itself remain intact. To 40 this end the binder filament is laid to form with the longitudinal axis of the conductor an angle  $b$  greater than the angle  $a$  formed therewith by the strands of the serving. As shown, angle  $b$  is approximately 65 degrees.

In Figs. III, IV and V of the drawing there is shown a complete conductor assembly in which the wrap 3, and binder structure 4, are shown as saturated with and embedded in an envelope 5 of viscous saturant, such as the pitchy moisture-resistant and flame-retardant material commonly used in making insulated conductors. In addition to this encapsulation of the viscous material, there are other layers of encapsulating material, such as paint and wax, which are designated by reference numerals 6 and 7.

Considering these figures of the drawing, it will be apparent how a separation of the served turns of the wrap, by breaking through the encapsulating coatings of the conductor and interrupting the cohesion of the wrap, exposes the rubber sheath 2 to deteriorating agencies, and will allow moisture to work into the interior of the conductor structure. It will similarly be apparent not only why the short lead of the binder 65 helix is of advantage in lessening elongation of the binder, but also how a binder of sufficient strength may continue to oppose the opening tendency by the turns of the served wrap during severe flexion by continuing to exert its binding 70 force as a reaction to the forced increase in its

length which flexion causes. That is, we have discovered that the yielding of the binder to flexion, by its elongation, does not temporarily so negative its binding effect as to permit the opening between turns of the wrap which must 75 be prevented.

It has been indicated that in order to obtain maximum life and utility of the insulated conductor, the angle or lead of the binder structure is of importance in protecting the binder structure against severe flexion. In smaller size conductors, such as the conductor shown in Fig. I of the drawing, more abrupt flexion angles are usually encountered, but with the larger size conductors, the effect of flexion is proportionally 15 greater, and this is particularly true in those turns of a large size conductor, which is so closely coiled as to be subjected to an elongating effect throughout a relatively great length of its binder helix. In Fig. II, therefore, the served wrap 3a 20 surrounding the conductor core has its strands or turns bound together by a filamentary binder structure 4a laid at an angle of approximately 70 degrees to the longitudinal axis of the conductor.

We have made an additional discovery which 25 in the insulated binder assembly is one of substantial importance. It is, that in the assembly the security of integration depends not only in the presence of the binder filament, but in the extensibility of that filament as applied to the 30 served wrapping which by its binding effect the binder structure maintains in coherent condition. Thus, if the binder filament be made of cotton, as is conventional there is in severe flexion of the conductor a frequently destructive tendency to 35 disrupt the binder at some point in its helical structure at which the forces tending to elongate the material of the helix exceed the ability of the material to elongate. As explained above, the angle at which the helical turns of the binder 40 structure are laid is of importance in modifying that tendency. We have found that if the helix of the open binder structure be of adequate extensibility, the binder structure may be greatly elongated without losing its effectiveness by a 45 loosening of its turns. That is, being able to resist rupture because of its extensibility and strength, it is enabled progressively so to react against the elongating forces that it continues effectively to bind the turns of the serving to 50 each other.

Taking as a standard for use specifically as binder filaments in the described assembly, the various filamented cellulose esters known generically by the trade name "Rayon", and the filamented fiber-forming high-molecular-weight polyamides known by the trade name "Nylon" and disclosed in United States Patents to Wallace H. Carothers No. 2,130,947 and No. 2,130,948, we have found that such materials exemplary of 60 those whose inherent viscosity permits them to be extruded into long individually strong and elastic fibers, have an extensibility, or elongation, and elastic recovery greatly exceeding that of cotton. For example, the extensibility or elongation of 65 the cellulose ester filaments is approximately three times that of a high grade cotton filament, coupled with a strength twice that of the cotton filament. The polyamide filaments have an extensibility, or elongation, about four times that 70 of a corresponding cotton filament coupled with a strength about twice that of the cotton filament. In these exemplary materials extensibility and strength are coupled, and we have found that when used in an insulated conductor assem- 75

bly as an open binder structure; such as the binder 4, filaments of this sort retain their effectiveness in binding the served wrap both during and following severe elongation. This is in distinction 5 from cotton which ruptures when its ability to elongate is quickly exhausted, and other materials which, while possessing marked extensibility, lose their ability to sustain loads when elongated.

10 In evaluating the benefit of extensibility in the open binder structure of a conductor organized as herein shown, in terms of improvement in the conductor assembly, we may say that a more specialized binder filament does not lead to striking improvement in the conductor assembly unless it has an extensibility greatly exceeding that of a similar binder structure made of the conventional cotton filament, and couples this with a strength greater than that of a binder structure 15 made of cotton filament. This, because the advantages derived from extensibility, does not progressively occur with increase in extensibility. Whereas the elongation in the conductor assembly may be effective throughout a relatively great 20 length of the conductor, it may be wholly localized, so that by a relatively short length of the binder filament is called upon to endure the forces tending by elongation to rupture it. We can, therefore, say that to obtain substantial 25 benefit in the conductor structure as a whole from the selective inclusion of an extensible binder filament, the binder filament must have a comparative extensibility almost twice that of the conventional cotton, and preferably should have an 30 extensibility as great as that of rayon.

35 The materials herein identified as "Rayon" and "Nylon" do not have an origin in common. Both may be considered as synthetic silk-like fibrous

materials, although "Rayon" is derived from cellulose, and "Nylon" is produced by reacting diamines with di-carboxylic acids or amine-forming derivatives of dibasic carboxylic acid. They are 5 representatives of a class of filamentary materials of like character, which also possess in common the quality of extensibility in high order and relatively great strength.

We claim as our invention:

1. An electrical conductor assembly comprising 10 an electrically insulated inner conductive structure and an outer protective jacket therefore in the form of a helical serving of highly absorbent and relatively inelastic thread laid in close turns with a substantial lead and without 15 overlap, to give approximately complete coverage and an effective saturant-absorbing assembly, in combination with an open locking structure composed of a filament of plastic material which is 20 substantially less absorbent and substantially stronger and more elastic than the thread of the absorbent jacket, said filament being wound upon the said absorbent jacket oppositely to the winding thereof and at a substantial angle with the conductor axis and with its turns so spaced as to 25 expose the greater part of said jacket.

2. An electrical conductor assembly in accordance with claim 1 in which the relatively strong and elastic locking filament of the assembly is a filament selected from the fiber-forming 30 cellulose esters.

3. An electrical conductor assembly in accordance with claim 1 in which the relatively strong and elastic locking filament of the assembly is composed of filamented fiberforming 35 super-polyamides.

WILLIAM C. ROBINSON.  
RALPH W. E. MOORE.